

## UNITED STATES PATENT OFFICE

RENÉ CLAVEL, OF BASEL-AUGST, NEAR BASEL, SWITZERLAND

## TREATMENT OF PRODUCTS OR GOODS OF OR CONTAINING CELLULOSE DERIVATIVES

No Drawing. Application filed January 14, 1926, Serial No. 81,322, and in Germany September 28, 1925.

This invention relates to improvements in the restoration of lustre to delustered threads, yarns, fabrics, or other products made of or containing cellulose acetate.

5 Cellulose acetate goods can be delustered by treatment in boiling soap baths or in acid baths. Thus by the use of baths containing an organic acid, woolly effects can be produced by a control of the concentration and 10 temperature of the bath and the duration of the treatment, the volume or bulk of the goods being increased to 3 to 5 times their original volume. In this way a lustrous cellulose acetate fabric can be converted into a fabric 15 that is both lustreless and more bulky in character. These lustreless fabrics, whether dyed or undyed, or containing other natural or artificial fibres, present an entirely new character approximating to that of woollen 20 goods. Hitherto it has been necessary, for the production of a figured fabric (partly lustrous and partly lustreless) to make a mixed fabric containing a textile material which is not affected by boiling soap 25 solutions or by acids. By this method, a figured fabric of an attractive character can be obtained, but the manufacture of the goods is expensive and complicated, and important economies would be effected if the same results could be produced by a simpler method. 30 This result could be obtained if after delustering the whole of the cellulose acetate goods it were possible to restore to a lustrous condition the part or parts constituting the 35 design, pattern or figure.

Again it sometimes happens that, owing to carelessness of the dyer in watching the concentration or temperature of the acid, part of the goods becomes delustered. A similar 40 defect sometimes arises from the goods coming into contact with the steam pipes used for heating purposes. Defective goods of this character are unsalable and a method of restoring partly delustered goods to a lustrous 45 condition would be of great value.

After many experiments it has been discovered that the lustre of cellulose acetate goods can be restored by the use of substances that are capable of forming a solution with 50 cellulose acetate (whether such solution be a

liquid solution or a solid solution), that is to say, substances which act as solvents or swelling agents for cellulose acetate, and afterwards steaming the goods preferably under pressure.

As solvents or swelling agents may be used the organic acids (acetic, formic, etc.) employed for delustering purposes, and also alcohols, esters and salt solutions, e. g. a solution of calcium sulphocyanide.

The steaming operation is preferably effected with aid of steam at a pressure in excess of the atmosphere. The pressures used may range up to 5 atmospheres absolute or even higher, always provided that the temperature is not so high as to melt or damage the cellulose acetate goods.

Apparently the relustered goods retain to a large extent the increased volume or bulk produced by the delustering process to which 70 they were first subjected.

Figured and other partly lustrous and partly lustreless goods of a very attractive character are produced by applying to a delustered fabric a printing paste or a stencil- 75 ling or like preparation containing a solvent or swelling agent, and afterwards steaming the goods, so that the fabrics are relustered at the parts to which the paste is applied. In this way, brilliant and effective designs or 80 figures may be produced on a dull ground. Dyes or mordants may be added to the relustering pastes so that different colour effects can also be obtained.

Relustering may also be effected by wholly 85 or partially immersing the goods, in, or otherwise treating the goods with, baths containing a solvent or swelling agent, to which may be added if desired dyestuffs, salts, mordants, or protective colloids, separately or in combination. After a suitable interval, the goods are removed, quickly dried and subjected to the action of steam.

Preferably, baths containing a weak solution of an organic acid are used, but if stronger solutions are used, the steaming operation may be shortened or even omitted, the goods being simply dried after removal from the bath.

In certain cases, notably where the cellu-

lose acetate fibre contains residual solvent, for example, when a solvent of high boiling point has been employed in the manufacture of the fibres, treatment with solvent or swelling agents may be omitted, and lustre may be restored by the application of steam alone to the delustered goods. A lustre can thus be obtained closely resembling that of natural silk, the goods nevertheless retaining to a large extent, the bulky or voluminous character imparted by the original delustering operation. In steaming defective goods, the relustering of the delustered parts is accompanied by partial delustering of the lustrous parts, so that goods of a uniform lustre are obtained, this effect being probably due to the fact that the steam used for relustering, though substantially free from water in the form of "condense" or mist, may, nevertheless, carry traces of water which can act as a delustering agent for the fully lusted portions of the goods until a state of equilibrium is reached. Of course, if steam carrying large quantities of "condense" or mist, that is to say, a mixture of steam and water, were applied to the fabric, it would act as a delustering agent in the same way as boiling water or boiling soap solutions.

*Example I*

30 Piece goods of delustered cellulose acetate are printed with a paste made by emulsifying together 650 grams of gum arabic (50%) with 300 cc. of ethyl alcohol and 15 grams of 35 Rhodulin orange. The printed goods are well dried, steamed at a pressure of 1.4 atmospheres absolute, and finally cold washed. The pattern then comes up as a lustrous figure on a lustreless ground.

40 *Example II*

Delustered cellulose acetate yarn in the form of hanks is partly immersed in a bath containing 0.5% of acetic acid, and maintained 45 at a temperature of 50° C. After one-half to one hour, the yarn is removed, centrifuged, dried and steamed for half an hour under pressure.

It will be understood that the process is not 50 limited to the procedure set forth in the preceding examples, but may be varied within wide limits without departing from the invention.

What I claim and desire to secure by Letters Patent is:—

55 1. A process of imparting lustre to delustered material comprising cellulose acetate and a substance capable of forming a solution with cellulose acetate, which comprises 60 subjecting the material to the action of dry steam.

2. A process of imparting lustre to delustered material comprising cellulose acetate, which comprises treating the material 65 with a substance capable of forming a solu-

tion with cellulose acetate, and afterwards subjecting the material to the action of dry steam.

3. A process of imparting lustre to delustered material comprising cellulose acetate, which comprises treating the material with an aqueous preparation containing a substance capable of forming a solution with cellulose acetate, and afterwards subjecting the material to the action of dry steam. 75

4. A process of imparting lustre to delustered material comprising cellulose acetate, which comprises treating the material with an aqueous solution containing a solvent for cellulose acetate, and afterwards subjecting the material to the action of dry steam. 80

5. A process for imparting lustre to delustered material comprising cellulose acetate, which comprises treating the material with an aqueous solution of acetic acid, and afterwards subjecting the material to the action of dry steam. 85

6. A process of imparting lustre to delustered material comprising cellulose acetate, which comprises treating the material with a substance capable of forming a solution with cellulose acetate, and afterwards drying the material and subjecting the same to the action of dry steam. 90

7. A process of imparting lustre to delustered material comprising cellulose acetate, which comprises treating the material with an aqueous preparation containing a substance capable of forming a solution with cellulose acetate, and afterwards drying the material and subjecting the same to the action of dry steam. 95

8. A process of imparting lustre to delustered material comprising cellulose acetate, which comprises treating the material with an aqueous solution of a solvent for cellulose acetate and afterwards drying the material and subjecting the same to the action of dry steam. 105

9. A process of imparting lustre to delustered material comprising cellulose acetate, which comprises treating the material with an aqueous solution of acetic acid, and afterwards drying the material and subjecting the same to the action of dry steam. 110

10. A process for the manufacture of figured and other lustrous effects on delustered cellulose acetate material, which comprises applying to selected areas of the delustered material a substance capable of forming a solution with cellulose acetate, and afterwards subjecting the material to the action of dry steam. 115

11. A process for the manufacture of figured and other lustrous effects on delustered cellulose acetate material, which comprises applying to selected areas of the delustered material an aqueous preparation containing a substance capable of forming a solution with cellulose acetate, and afterwards sub- 120

jecting the material to the action of dry steam.

12. A process for imparting a lustre resembling that of natural silk to yarns, threads, fabrics or other material comprising delustrated cellulose acetate filaments containing a substance capable of forming a solution with cellulose acetate, which comprises subjecting the material to the action of dry steam.

10 In testimony whereof I have hereunto subscribed my name.

RENE CLAVEL.

.5

20

25

30

35

40

45

50

55

60

65